# EUROPEAN PATENT SPECIFICATION

(11) **EP 2 415 887 B1**
(45) Date of publication and mention of the grant of the patent: **10.02.2016**
(21) Application number: 10758330.4
(22) Date of filing: 17.02.2010
(51) Int. Cl.: C22C 9/06, C22F 1/08, H01B 1/02, C22F 1/00, C22F 1/02

(54) **CU-CO-SI COPPER ALLOY FOR USE IN ELECTRONICS, AND MANUFACTURING METHOD THEREFOR**
CU-CO-SI-KUPFERLEGIERUNG FÜR DIE ELEKTRONIK UND HERSTELLUNGSVERFAHREN DAFÜR
ALLIAGE DE CUIVRE À BASE DE CUIVRE, DE COBALT ET DE SILICIUM DESTINÉ À ÊTRE UTILISÉ DANS L'ÉLECTRONIQUE, ET PROCÉDÉ DE FABRICATION DE CET ALLIAGE

(30) Priority: 31.03.2009 JP 2009088287
(43) Date of publication of application: 08.02.2012
(73) Proprietor: JX Nippon Mining & Metals Corporation, Chiyoda-ku Tokyo 100-0004 (JP)
(72) Inventor: ONDA,Takuma, Hitachi-shi Ibaraki 317-0056 (JP); KUWAGAKI,Hiroshi, Hitachi-shi Ibaraki 317-0056 (JP)
(74) Representative: Banse & Steglich
(86) International application number: PCT/JP2010/052375
(87) International publication number: WO 2010/113553

(56) References cited:
- EP-A1- 1 873 267
- WO-A1-2009/148101
- JP-A- 9 020 943
- JP-A- 9 020 943
- JP-A- 2007 246 931
- JP-A- 2008 088 512
- JP-A- 2008 088 512
- JP-A- 2008 266 783
- JP-A- 2008 266 783
- JP-A- 2010 059 543
- US-A1- 2004 079 456
- VARSCHAVSKY ARI ET AL: "Influence of microstructure on the subcritical crack growth in Cu-Co-Si alloys", CONGRESSO ANUAL - ASSOCIACAO BRASILEIRA DE METALURGIA E MATERIAIS,, vol. 2, 1 January 1995 (1995-01-01), pages 503-510, XP009168540,

## Description

### FIELD OF THE INVENTION

The present invention relates to precipitation hardening copper alloys, in particular, to Cu-Co-Si system alloys suitable for use in a variety of electronic components.

### BACKGROUND OF THE INVENTION

A copper alloy for electronic materials that are used in a connector, switch, relay, pin, terminal, lead frame, and various other electronic components is required to satisfy both high strength and high electrical conductivity (or thermal conductivity) as basic characteristics. In recent years, as high integration and reduction in size and thickness of an electronic component have been rapidly advancing, requirements for copper alloys used in these electronic components have been increasingly becoming severe.

Because of considerations related to high strength and high electrical conductivity, the amount in which precipitation-hardened copper alloys are used has been increasing, replacing conventional solid-solution strengthened copper alloys typified by phosphor bronze and brass as copper alloys for electronic components. With a precipitation-hardened copper alloy, the aging of a solution-treated supersaturated solid solution causes fine precipitates to be uniformly dispersed and the strength of the alloys to increase. At the same time, the amount of solved elements in the copper is reduced and electrical conductivity is improved. For this reason, it is possible to obtain materials having excellent strength, spring property, and other mechanical characteristics, as well as high electrical and thermal conductivity.

Among precipitation hardening copper alloys, Cu-Ni-Si system alloys commonly referred to as Corson alloys are typical copper alloys having relatively high electrical conductivity, strength, and bending workability, and are among the alloys that are currently being actively developed in the industry. In these copper alloys, fine particles of Ni-Si intermetallic compounds are precipitated in the copper matrix, thereby increasing strength and electrical conductivity.

Various experiments have been made with the aim of further improving the characteristics of Corson alloys by adding Co.

Patent document 1 discloses that Co is similar to Ni in forming a compound with Si and increasing mechanical strength, and when Cu-Co-Si system alloys are aged, they have better mechanical strength and electrical conductivity than Cu-Ni-Si system alloys, and where acceptable in cost, Cu-Co-Si system alloys may be also selected. The document also discloses that the optimum additive amount of Co is 0.05 to 2.0 wt%.

Patent document 2 discloses that cobalt content should be 0.5 to 2.5 wt% because the precipitation of the cobalt-containing silicide as second-phase is insufficient when the cobalt content is less than 0.5 wt%, and excessive second-phase particles precipitate, formability is reduced, and the copper alloy is endowed with undesirable ferromagnetic properties when the cobalt content exceeds 2.5 wt%. The document discloses that the cobalt content is preferably about 0.5 wt% to about 1.5 wt%, and the cobalt content is about 0.7 wt% to about 1.2 wt% in the most preferable embodiment.

Copper alloys disclosed in Patent document 3 have been developed with the aim of applications mainly for an end terminal of vehicle installation, communication instrument, and the like, or connector materials. The copper alloys are Cu-Co-Si system alloys in which cobalt concentration is 0.5 to 2.5 wt% and high electrical conductivity and moderate strength are achieved. The document discloses that the cobalt concentration is limited within the above described range because desirable strength cannot be provided when additive amount of cobalt is less than 0.5 wt%, and high strength can be provided, but electrical conductivity remarkably deteriorates and further hot processing characteristics deteriorates when cobalt concentration exceeds 2.5 wt%. The document discloses that the cobalt concentration is preferably 0.5 to 2.0 wt%.

Copper alloys disclosed in Patent document 4 have been developed with the aim of achieving high strength, high electrical conductivity and high bending workability and limit cobalt concentration to 0.1 to 3.0 wt%. The document discloses that the cobalt concentration is limited within the above described range because it is undesirable that the alloys do not have the above described effects when the cobalt concentration is less than the range, and the crystallized phase is generated at casting and it leads to breaks at casting when the cobalt concentration exceeds the range.
[Patent document 1] Japanese patent laid-open publication No. 11-222641
[Patent document 2] Japanese Domestic Republication No. 2005-532477
[Patent document 3] Japanese patent laid-open publication No. 2008-248333
[Patent document 4] Japanese patent laid-open publication No. 9-20943

### SUMMARY OF THE INVENTION

### PROBLEMS TO BE SOLVED BY THE INVENTION

Though it is known that the addition of Co contributes to an improvement of copper alloys properties as discussed previously, having Co in high concentration negatively affects manufacturing properties and alloys properties as disclosed in the above prior documents, and improvements of Cu-Co-Si system alloys properties in which cobalt is added in high concentration have not been discussed sufficiently. However, Co improves mechanical strength and electrical conductivity more than Ni, and then possibility that Cu-Co-Si system alloys properties can be improved by increasing Co concentration more is considered to remain. On the other hand, to increase Co concentration more requires an operation of a solution treatment at higher temperature. In such cases, recrystallized grains are liable to increase in size. Further, secondary-phase particles such as crystalloid components and precipitated components precipitated before the solution treatment step act as obstacles and block grain growth. Accordingly, ununiformity of recrystallized grains in alloys increases and a problem of increase on a variability of mechanical characteristics of alloys occurs.

The object of the invention is to provide Cu-Co-Si system alloys containing high concentration Co, having high electrical conductivity, high strength and high bending workability, and having uniform mechanical characteristics. Another object of the invention is to provide a method for manufacturing such Cu-Co-Si system alloys.

### MEANS FOR SOLVING THE PROBLEM

The inventors have diligently studied means for decrease in variability of recrystallized gains, and eventually have found out that, in a manufacturing process for Cu-Co-Si system alloys that contain Co in high concentration, when the solution treatment is conducted in relatively-high temperature, the grain size does not increase so much because of pinning effect of the second-phase particles and the pinning effect works evenly in an entire copper base matrix, resulting in uniformalization of the size of growing recrystallized grains by precipitating fine second-phase particles in copper base matrix as equally spaced apart and uniformly as possible before the solution treatment step. As a result, Cu-Co-Si system alloys having small variability of mechanical characteristics can be provided.

Subject of the invention is a copper alloy for electronic materials according to claim 1, a method according to claim 2, a copper alloy product of claim 3 and an electronic component of claim 4.

In one aspect, the present invention that has been made based on these findings is a copper alloy for electronic materials, containing 0.5 to 4.0 mass% Co, 0.1 to 1.2 mass% Si, the balance being Cu and unavoidable impurities, wherein an average grain size is 15 to 30 µm and an average difference between maximum grain size and minimum grain size in every observation field of 0.5 mm² is not more than 7 µm.

In another aspect, the present invention is the copper alloy wherein Cr is furthermore contained in a maximum amount of 0.5 mass%.

In an embodiment, the present invention is the copper alloy wherein a single element or two or more elements selected from Mg, Mn, Ag and P are furthermore contained in total in a maximum amount of 0.5 mass%.

In another embodiment, the present invention is the copper alloy wherein one or two elements selected from Sn and Zn are furthermore contained in total in a maximum amount of 2.0 mass%.

In a further embodiment, the present invention is the copper alloy wherein a single element or two or more elements selected from As, Sb, Be, B,Ti, Zr, Al and Fe are furthermore contained in total in a maximum amount of 2.0 mass%.

In a further aspect, the present invention is a method for manufacturing the copper alloy, comprising sequentially conducting:
- step 1 for casting an ingot having a desired composition;
- step 2 for heating the ingot for not less than 1 hour at 950 °C to 1050 °C, thereafter hot rolling the ingot, setting the temperature to not less than 850 °C when hot rolling is completed, and cooling the ingot at an average cooling rate being not less than 15 °C/s from 850 °C to 400 °C;

- step 3 for cold rolling at a reduction ratio being not less than 70 %;
- step 4 for conducting aging by heating at 350 °C to 500 °C for 1 to 24 hours;
- step 5 for conducting a solution treatment at 950 °C to 1050 °C, for 60 to 300 seconds at not less than 950 °C to less than 1000 °C, and for 30 to 180 seconds at not less than 1000 °C to less than 1050 °C, and cooling the material at an average cooling rate being not less than 15 °C/s when the material temperature is reduced from 850 °C to 400 °C;
- step 6 for conducting optional cold rolling;
- step 7 for conducting aging; and
- step 8 for conducting optional cold rolling.

In a further aspect, the present invention is a copper alloy product using the copper alloy according to the present invention.

In a further aspect, the present invention is an electronic component using the copper alloy according to the present invention.

### ADVANTAGEOUS EFFECT OF THE INVENTION

The invention can provide Cu-Co-Si system alloys that have desirable mechanical and electrical characteristics as a copper alloy for electronic materials, and have uniform mechanical characteristics.

### BRIEF DESCRIPTION OF THE FIGURES

Fig.1 is an illustration to explain the method of the stress relaxation test.
Fig.2 is an illustration to explain the amount of permanent set in the method of the stress relaxation test.

### PREFERRED EMBODIMENT OF THE INVENTION

### (Additive amount of Co and Si)

Co and Si form an intermetallic compound with appropriate heat-treatment, and make it possible to increase strength without adversely affecting electrical conductivity.

When the additive amount of Co and Si are such that Co is less than 0.5 mass% and Si is less than 0.1 mass% respectively, the desired strength cannot be achieved, and conversely, when the additive amount of Co and Si are such that Co is more than 4.0 mass% and Si is more than 1.2 mass% respectively, higher strength can be achieved, but electrical conductivity is dramatically reduced and hot workability furthermore deteriorates. Therefore, the additive amounts of Co and Si are such that Co is 0.5 to 4.0 mass% and Si is 0.1 to 1.2 mass% in the present invention.

The high strength is more desired in Cu-Co-Si system alloys than in Cu-Ni-Si system alloys and in Cu-Ni-Si-Co system alloys. Therefore, the high concentration of Co is desired and the concentration of Co is preferably not less than 2.5 mass%, more preferably not less than 3.2 mass%. That is, the additive amounts of Co and Si are such that, preferably, Co is 2.5 to 4.0 mass% and Si is 0.5 to 1.0 mass%, and more preferably, Co is 3.2 to 4.0 mass% and Si is 0.65 to 1.0 mass%.

### (Additive amount of Cr)

Cr preferentially precipitates along crystal grain boundaries in the cooling process at the time of casting. Therefore, the grain boundaries can be strengthened, cracking during hot rolling is less liable to occur, and a reduction in yield can be limited. That is, Cr that has precipitated along the grain boundaries during casting is solved again by solution treatment and the like, resulting in producing precipitated particles or compounds with Si, having a bcc structure mainly composed of Cr in the subsequent aging precipitation. With an ordinary Cu-Ni-Si system alloy, the portion of the added Si solved in the matrix, which has not contributed to aging precipitation, suppresses an increase in electrical conductivity, but the Si content solved in the matrix can be reduced and electrical conductivity can be increased without compromising strength by adding Cr as a silicide-forming element and causing silicide to further precipitate. However, when the Cr concentration exceeds 0.5 mass%, coarse second-phase particles are more easily formed and product characteristics are compromised. Therefore, in the Cu-Co-Si system alloys according to the present invention, Cr can be added in a maximum amount of 0.5 mass%. However, since the effect of the addition is low at less than 0.03 mass%, it is preferred that the additive amount be 0.03 to 0.5 mass%, and more preferably 0.09 to 0.3 mass%.

### (Additive amount of Mg, Mn, Ag and P)

The addition of traces of Mg, Mn, Ag and P can improve strength, stress relaxation characteristics, and other manufacturing characteristics without compromising electrical conductivity. The effect of the addition is mainly produced by the formation of a solid solution in the matrix, but the effect can be further produced when the elements are contained in the second-phase particles. However, when the total concentration of Mg, Mn, Ag and P exceeds 0.5 masss%, the effect of improving the characteristics becomes saturated and manufacturability is compromised. Therefore, in the Cu-Co-Si system alloys according to the present invention, a single element or two or more elements selected from Mg, Mn, Ag and P can be added in total in a maximum amount of 0.5 mass%. However, since the effect of the addition is low at less than 0.01 mass%, it is preferred that the additive amount be a total of 0.01 to 0.5 mass%, and more preferably a total of 0.04 to 0.2 mass%.

### (Additive amount of Sn and Zn)

The addition of traces of Sn and Zn also improves the strength, stress relaxation characteristics, plating properties, and other product characteristics without compromising electrical conductivity. The effect of the addition is mainly produced by the formation of a solid solution in the matrix. However, when the total amount of Sn and Zn exceeds 2.0 mass%, the characteristics improvement effect becomes saturated and manufacturability is compromised. Therefore, in the Cu-Co-Si system alloys according to the present invention, one or two elements selected from Sn and Zn can be added in total in a maximum amount of 2.0 mass%. However, since the effect of the addition is low at less than 0.05 mass%, it is preferred that the additive amount be a total of 0.05 to 2.0 mass%, and more preferably a total of 0.5 to 1.0 mass%.

### (Additive amount of As, Sb, Be, B,Ti, Zr, Al and Fe)

Electrical conductivity, strength, stress relaxation characteristics, plating properties, and other product characteristics are improved by adjusting the additive amount of As, Sb, Be, B,Ti, Zr, Al and Fe in accordance with the required product characteristics. The effect of the addition is mainly produced by the formation of a solid solution in the matrix, but a further effect can be produced when the above-described elements are added to the second-phase particles or when second-phase particles having a new composition are formed. However, when the total concentration of these elements exceeds 2.0 mass%, the characteristics improvement effect becomes saturated and manufacturability is compromised. Therefore, in the Cu-Co-Si system alloys according to the present invention, a single element or one or greater elements selected from As, Sb, Be, B,Ti, Zr, Al and Fe can be added in total in a maximum amount of 2.0 mass%. However, since the effect of the addition is low at less than 0.001 mass%, it is preferred that the additive amount be a total of 0.001 to 2.0 mass%, and more preferably a total of 0.05 to 1.0 mass%.

Manufacturability is readily compromised when the additive amount of the Mg, Mn, Ag, P, Sn, Zn, As, Sb, Be, B,Ti, Zr, Al and Fe described above exceeds 3.0 mass% as a total. Therefore, it is preferred that the total be not more than 2.0 mass%, and more preferably not more than 1.5 mass%

### (Grain size)

Hall-Petch rule in which a crystal grain has an influence on the strength and the strength is proportional to (the grain size)^{-1/2} is generally effected. Further, a coarse crystal grain deteriorates bending workability and it triggers rough surface at bending work. Accordingly, a refinement of the crystal grain is generally desirable for an improvement of strength of copper alloys. In particular, the crystal grain is preferably not more than 30 µm, and more preferably not more than 23 µm.

On the other hand, Cu-Co-Si system alloys according to the present invention are precipitation-hardened copper alloys, and then it is also necessary to note precipitation state of second-phase particles. The second-phase particles precipitated in the crystal grain at aging treatment endow improvement of strength of copper alloys. However, the second-phase particles precipitated in the crystal grain boundary hardly endow improvement of strength of copper alloys. Therefore, in order to improve strength of copper alloys, it is desirable to precipitate the second-phase particles in the crystal grain. When the grain size decreases, the crystal grain boundary area increases. Accordingly, the second-phase particles become easy to be precipitated preferentially in the crystal grain boundary at aging treatment. In order to precipitate the second-phase particles in the crystal grain, it is necessary that the crystal grain has a certain level of size. In particular, the grain size is preferably not less than 15µm, and more preferably not less than 18 µm.

In the present invention, the average grain size is controlled within the range of 15 to 30 µm. The average grain size is preferably 18 to 23 µm. By controlling the average grain size within such a range, both the improvement effects of strength caused by the refinement of crystal grain and caused by the precipitation hardening can be achieved in a balanced manner. Further, when the average grain size is within the range, excellent bending workability and stress relaxation characteristics can be provided.

In the present invention, the grain size indicates a diameter of a minimum circle surrounding individual crystal grain, being provided by a microscope observation of a cross-section surface in the thickness direction parallel to the rolling direction. The average grain size indicates an average amount of those grain sizes.

In the present invention, an average difference between maximum grain size and minimum grain size in every observation field of 0.5 mm² is not more than 7 µm. Though the average difference is ideally 0 µm, it is realistically difficult to be achieved. Therefore, a lower limit of the average difference is 3µm from an actual minimum value, and typically 3 to 7 µm is optimum. The maximum grain size indicates a maximum grain size observed in an observation field of 0.5 mm². The minimum grain size indicates a minimum grain size observed in the same observation field. In the present invention, differences between maximum grain size and minimum grain size are measured in 15 observation fields, and an average value of the differences indicates the average difference between maximum grain size and minimum grain size.

The crystal grain size is uniform when the difference between maximum grain size and minimum grain size is small, and then variability of mechanical characteristics at every measuring point in the same materials is reduced. As a result, quality stability of copper alloy products or electronic components produced by using copper alloys of the present invention is improved.

### (Method for manufacturing)

In a general manufacturing process, which does not belong to the present invention, for Corson copper alloys, firstly, electrolytic cathode copper, Si and Co, and other starting materials are melted in a atmospheric melting furnace to obtain a molten metal having the desired composition. Then the molten metal is cast in a mold to produce an ingot. Hot rolling is conducted thereafter, cold rolling and heat treatment are repeated, and a strip or a foil having a desired thickness and characteristics are finished. The heat treatment includes solution treatment and aging treatment. In the solution treatment, material is heated at a high temperature of about 700 to about 1000 °C, the second-phase particles are solved in the Cu base matrix, and the Cu base matrix is simultaneously re-crystallized. Hot rolling sometimes doubles as the solution treatment. In an aging treatment, material is heated for not less than 1 hour in a temperature range of about 350 to about 550 °C, and second-phase particles formed into a solid solution in the solution treatment are precipitated as microparticles on a nanometer order. The aging treatment results in increased strength and electrical conductivity. Cold rolling is sometimes performed before and/or after the aging treatment in order to obtain higher strength. Further, stress relief annealing (low-temperature annealing) is sometimes performed after cold rolling in the case that cold rolling is conducted after aging.

Grinding, polishing, shot blast pickling and the like may be conducted as needed in order to remove oxidized scale on the surface between each of the above-described steps.

The manufacturing process described above is also used basically in the copper alloys according to the present invention, but the process of the present invention is defined by claim 2, and it is important to precipitate fine second-phase particles in copper base matrix as equally spaced and uniformly as possible before the solution treatment step as described above in order to control the average grain size and the variability of grain size within the range as defined in the present invention. In order to provide copper alloys according to the present invention, it is necessary to produce them with particular attention to the following points.

First, coarse crystallites are unavoidably generated in the solidification process at the time of casting, and coarse precipitates are unavoidably generated in the cooling process. Therefore, the crystallites must form a solid solution in the matrix in the steps that follow. The material is held for not less than 1 hour at 950 °C to 1050 °C and then subjected to hot rolling, and when the temperature at the end of hot rolling is set to not less than 850 °C, a solid solution can be formed in the matrix even when Co, and Cr as well, are added. The temperature condition of not less than 950 °C is a higher temperature setting than in the case of other Corson alloys. When the holding temperature before hot rolling is less than 950 °C, solid solution is not sufficient. When the holding temperature before hot rolling exceeds 1050 °C, the material may melt. When the temperature at the end of hot rolling is less than 850 °C, it is difficult to obtain high strength because the elements, which have formed a solid solution, will precipitate again. Therefore, it is preferred that hot rolling be ended at 850 °C and the material be rapidly cooled in order to obtain high strength.

In this process, when the cooling rate is low, Si system compounds containing Co and Cr are precipitated again. When a heating treatment (aging treatment) is conducted in such compositions with the aim of improvement of strength, precipitates in the cooling process become growth cores, and coarse precipitates which do not contribute to strength grow from the cores, and then high strength cannot be provided. Accordingly, it is necessary that the cooling rate should be as high as possible, in particular, not less than 15 °C/s. However, the secondary-phase particles remarkably precipitates until the temperature increases to about 400 °C, and then the cooling rate in the temperature of less than 400 °C does not make any difference. Therefore, in the present invention, the cooling is conducted at the average cooling rate of not less than 15 °C/s, preferably not less than 20 °C/s when the material temperature is reduced from 850 °C to 400 °C. "The average cooling rate when the material temperature is reduced from 850 °C to 400 °C" indicates a value (°C/s) being calculated by a formula of "(850-400) (°C)/cooling time (s)", wherein the cooling time is measured as time when the material temperature is reduced from 850 °C to 400 °C.

Water cooling is the most effective method for increasing the cooling rate. However, the cooling rate can be increased by managing the water temperature because the cooling rate varies due to the temperature of the water to be used for water-cooling. The water temperature is preferably kept at not more than 25 °C because the desired cooling rate sometimes cannot be achieved when the water temperature is not less than 25 °C. When the material is placed in a tank filled with water, the temperature of the water readily increases to not less than 25 °C. Therefore, it is preferred that a spray (shower or mist) be used or cold water be constantly allowed to flow into the water tank to prevent the water temperature from increasing, so that the material is cooled at a constant water temperature (not more than 25 °C). The cooling rate can be increased by providing additional water-cooling nozzles or increasing the flow rate of water per unit of time.

The cold rolling is conducted after the hot rolling. The cold rolling is conducted with the aim of increasing strains which will be precipitation sites in order to generate precipitates uniformly. The cold rolling is preferably conducted at reduction rate of not less than 70 %, and more preferably not less than 85 %. When the cold rolling is not conducted and the solution treatment is conducted just after the hot rolling, precipitates cannot be generated uniformly. A combination of the hot rolling and the subsequent cold rolling may be repeated accordingly.

The first aging treatment is conducted after the cold rolling. If the secondary-phase particles remain before conducting the step, such secondary-phase particles grow further when the step is conducted, and then the sizes of the secondary-phase particles is different from those of secondary-phase particles which are generated first in the step. However, in the present invention, fine secondary-phase particles can be precipitated in uniform size and uniformly because remaining secondary-phase particles are discreated in the former step.

When the aging temperature of the first aging treatment is too low, however, precipitation amount of the secondary-phase particles providing pinning effect decreases and pinning effect generated in the solution treatment can be provided partially. Accordingly, the sizes of the crystal grains vary. On the other hand, when the aging temperature is too high, the secondary-phase particles become coarse and precipitate ununiformly, and then the sizes of the crystal grains vary. Further, the longer the aging time is, the larger the secondary-phase particles grow, and then it is necessary to set the aging time appropriately.

The first aging treatment is conducted at 350 to 500 °C for 1 to 24 hours, preferably at not less than 350 °C to less than 400 °C for 12 to 24 hours, at not less than 400 °C to less than 450 °C for 6 to 12 hours, and at not less than 450 °C to less than 500 °C for 3 to 6 hours, and then fine secondary-phase particles can be precipitated uniformly in the matrix. In such compositions, the growth of recrystallized grains generated in the solution treatment of the next step can be pinned uniformly, and then refined grain compositions having little variability of grain size can be provided.

The solution treatment is conducted after the first aging treatment. In this treatment, fine and uniform recrystallized grains are grown with a solid solution of the second-phase particles. Accordingly, it is necessary that the temperature of the solution treatment is 950 to 1050 °C. In this treatment, the recrystallized grams grow first and then the second-phase particles precipitated in the first aging treatment form solid solution. Accordingly, the growth of the recrystallized grains can be controlled by the pinning effect However, the pinning effect disappears after the second-phase particles form the solid solution, and then the recrystallized grains grow when the solution treatment is conducted for a long time. Therefore, the solution treatment time is 60 to 300 seconds at not less than 950 °C to less than 1000 °C, preferably 120 to 180 seconds, and 30 to 180 seconds at not less than 1000 °C to less than 1050 °C, preferably 60 to 120 seconds.

Also in the cooling step after the solution treatment, the average cooling rate in the material temperature being reduced from 850 °C to 400 °C should be not less than 15 °C/s, preferably not less than 20 °C/s in order not to precipitate the second-phase particles.

The second aging treatment is conducted after the solution treatment. Conditions of the second aging treatment may be such that are generally used because of their availability for refinement of the precipitates. However, it is necessary to note that the temperature and time should be set so that the precipitates may not coarsen. The aging conditions are, for example, the temperature is in the range of 350 to 550 °C, and the time is 1 to 24 hours, more preferably the temperature is in the range of 400 to 500 °C and the time is 1 to 24 hours. In addition, the cooling rate after the aging treatment has little influences on small or large for sizes of the precipitates. The cold rolling may be conducted before and/or after the second aging treatment. Before conducting the second aging treatment, precipitation sites may be increased and age hardening may be advanced by using the precipitation sites in order to improve strength. After conducting the second aging treatment, work hardening may be advanced by using the precipitates in order to improve strength.

The Cu-Co-Si system alloys according to the present invention can be used to produce various wrought copper alloy products, for example, plates, strips, tubes, rods, and wires. Further, the Cu-Co-Si system alloys according to the present invention can be used in lead frames, connectors, pins, terminals, relays, switches, foil material for secondary batteries, and other electronic components and the like.

### EXAMPLES

Hereinafter, working examples will be described with comparative examples in order to understand the present invention and advantages thereof better. However, the present invention is not limited to these examples.

Copper alloys having the compositions shown in Table 1 (working examples) and Table 2 (comparative examples) were melted in a high-frequency melting furnace at 1300 °C and then cast in a mold to produce ingots having a thickness of 30 mm. Next, the ingots were heated to 1000 °C, hot rolled thereafter to a plate thickness of 10 mm at finishing temperature (the temperature at the completion of hot rolling) of 900 °C, water-cooled to 850 °C to 400 °C at average cooling rate of 18 °C/s after the completion of hot rolling, and then cooled by being left in the atmosphere. Next, the metals were faced to a thickness of 9 mm in order to remove scales from the surface, and sheets having a thickness of 0.15 mm were then formed by cold rolling. First aging treatment was subsequently conducted at various aging temperatures for 3 to 12 hours (this aging treatment was not conducted on some of comparative examples), and then solution treatment was conducted at various temperatures for 120 seconds, and immediately water-cooled to 850 °C to 400 °C at average cooling rate of 18 °C/s, and then cooled by being left in the atmosphere. The sheets were then cold rolled to 0.10 mm, subjected to second age treatment in an inert atmosphere at 450 °C for 3 hours, and lastly cold rolled to 0.08 mm to produce test pieces.

The following various evaluation tests were conducted on the provided test pieces.

### (1) Average grain size

Resin filling was conducted to the test pieces in such a manner that their observation surfaces were cross-section surfaces in the thickness direction parallel to the rolling direction, and mirror finish was conducted on the observation surfaces by mechanical polish. Next, solution was prepared by blending hydrochloric acid and water by a ratio of 10 volume parts of hydrochloric acid of 36 % to 100 volume parts of water, and then ferric chloride having weight of 5% of the solution weight was dissolved to the solution. The test pieces were immersed in the prepared solution for 10 seconds, and then metal structures appeared. Next, the metal structures were magnified 100 times by an optical microscope, pictures of their observation fields of 0.5 mm² were taken, each diameter of minimum circle surrounding individual crystal grain was measured, and then mean value was calculated on every observation field. The average grain size is mean value of the grain sizes in 15 observation fields.

### (2) Average difference between maximum grain size and minimum grain size

With respect to measured grain sizes which were provided in measuring the average grain size, differences between maximum and minimum were measured in every observation field. The average difference between maximum grain size and minimum grain size is mean value of the differences in 15 observation fields.

### (3) Strength

With respect to strength, a tensile test was conducted in the rolling direction, and 0.2 % yield strength (YS:MPa) was measured. Variability of strength according to measurement spots corresponds to a difference between maximum strength and minimum strength of 30 points. The average strength is mean value of strengths in these 30 points.

### (4) Electrical conductivity

Electrical conductivity (EC:% IACS) was determined by measuring volume resistivity with the aid of double bridge. Variability of electrical conductivity according to measurement spots corresponds to a difference between maximum electrical conductivity and minimum electrical conductivity of 30 points. The average electrical conductivity is mean value of electrical conductivities in these 30 points.

### (5) Stress relaxation performance

In measuring the stress relaxation performance, as described in Fig.1, bending stress was loaded to each test piece processed to width: 10 mm and length: 100 mm and thickness (t):0.08 mm in the condition that gauge length (l) is 25 mm and height (y₀) is determined to be such that load stress is 80 % of 0.2 % yield strength. Next, the test pieces were heated at 150 °C for 1000 hours and then the amounts of permanent set (height: y) as described in Fig.2 were measured and the stress relaxation performances {[1 - (y - yₗ) (mm) / (y₀-yₗ) (mm)] × 100 (%)} were calculated. In addition, yₗ indicates height of an initial warpage before loading stress. Variability of stress relaxation performance according to measurement spots corresponds to a difference between maximum stress relaxation performance and minimum stress relaxation performance of 30 points. The average stress relaxation performance is mean value of stress relaxation performances in these 30 points.

### (6) Bending workability

Bending workability was measured by a surface roughness of bending part. W bending test was conducted to Bad Way (BW: a direction where the bending axis is parallel to the rolling direction) with reference to JIS-H3130. Then the surface of the bending part was analyzed by a confocal laser scanning microscope and Ra (µm) regulated in JIS-B0601 was calculated. Variability of roughness of bending according to measurement spots corresponds to a difference between maximum Ra and minimum Ra of 30 points. The average roughness of bending is mean value of Ra in these 30 points.

**(Table 1-1)**

| No. | composition (mass%) | | | | aging temperature (°C) | solution treatment temperature (°C) | average grain size (*µ*m) | max grain size - min grain size | average strength (MPa) | average electrical conductivity (%IACS) | average stress relaxation performance (%) | average roughness of bending (*µ*m) | variability of strength (MPa) | variability of stress relaxation performance (%) | variability of roughness of bending (*µ*m) |
|---|---|---|---|---|---|---|---|---|---|---|---|---|---|---|---|
| | Co | Si | Cr | others | | | | | | | | | | | |
| 1 | 0.7 | 0.17 | | | 450 | 950 | 17 | 7 | 675 | 62 | 82 | 1.70 | 25 | 2.6 | 0.55 |
| 2 | 0.7 | 0.17 | 0.2 | | 450 | 950 | 15 | 8 | 671 | 63 | 81 | 1.82 | 28 | 2.5 | 0.67 |
| 3 | 2.0 | 0.48 | 0 | 0 | 450 | 1020 | 23 | 8 | 777 | 57 | 82 | 2.14 | 30 | 3.8 | 0.67 |
| 4 | 2.0 | 0.48 | 0 | 0 | 500 | 1020 | 19 | 9 | 776 | 56 | 84 | 2.05 | 36 | 2.4 | 0.68 |
| 5 | 2.0 | 0.48 | 0.2 | 0 | 450 | 1020 | 19 | 5 | 788 | 58 | 83 | 2.13 | 37 | 3.1 | 0.71 |
| 6 | 2.0 | 0.48 | 0.2 | 0 | 500 | 1020 | 19 | 6 | 785 | 58 | 85 | 2.12 | 28 | 2.8 | 0.64 |
| 7 | 3.0 | 0.71 | 0 | 0 | 350 | 1020 | 25 | 8 | 867 | 53 | 86 | 2.06 | 43 | 3.5 | 0.90 |
| 8 | 3.0 | 0.71 | 0 | 0 | 400 | 1020 | 25 | 8 | 867 | 52 | 82 | 2.11 | 35 | 3.1 | 0.79 |
| 9 | 3.0 | 0.71 | 0 | 0 | 450 | 1020 | 18 | 6 | 861 | 50 | 85 | 2.08 | 39 | 3.7 | 0.77 |
| 10 | 3.0 | 0.71 | 0 | 0 | 500 | 1020 | 17 | 6 | 863 | 50 | 83 | 2.15 | 36 | 3.7 | 0.74 |
| 11 | 3.0 | 0.71 | 0 | 0 | 450 | 1050 | 22 | 7 | 902 | 52 | 82 | 2.24 | 38 | 2.8 | 0.82 |
| 12 | 3.0 | 0.71 | 0 | 0 | 500 | 1050 | 19 | 9 | 900 | 52 | 82 | 2.12 | 37 | 3.0 | 0.75 |
| 13 | 3.0 | 0.71 | 0 | 0.1 Mg | 450 | 1020 | 16 | 6 | 890 | 50 | 90 | 2.22 | 40 | 3.1 | 0.74 |
| 14 | 3.0 | 0.71 | 0 | 0.1 Mg | 500 | 1020 | 15 | 7 | 891 | 50 | 87 | 2.18 | 39 | 3.0 | 0.70 |
| 15 | 3.0 | 0.71 | 0 | 0.1 Mg | 450 | 1050 | 19 | 7 | 931 | 50 | 89 | 2.31 | 38 | 4.2 | 0.84 |
| 16 | 3.0 | 0.71 | 0 | 0.1 Mg | 500 | 1050 | 18 | 9 | 928 | 48 | 87 | 2.05 | 31 | 2.0 | 0.67 |
| 17 | 3.0 | 0.71 | 0.2 | 0 | 350 | 1020 | 21 | 8 | 877 | 53 | 86 | 2.32 | 45 | 3.6 | 0.79 |
| 18 | 3.0 | 0.71 | 0.2 | 0 | 400 | 1020 | 21 | 6 | 891 | 54 | 86 | 2.22 | 40 | 3.8 | 0.81 |

**(Table 1-2)**

| No. | composition (mass%) | | | | aging temperature (°C) | solution treatment temperature (°C) | average grain size (*µ*m) | max grain size -min grain size (um) | average strength (MPa) | average electrical conductivity (%IACS) | average stress relaxation performance (%) | average roughness of bending (*µ*m) | variability of strength (MPa) | variability of stress relaxation performance (%) | variability oaf roughness of bending (*µ*m) |
|---|---|---|---|---|---|---|---|---|---|---|---|---|---|---|---|
| | Co | Si | Cr | others | | | | | | | | | | | |
| 19 | 3.0 | 0.71 | 02 | 0 | 450 | 1020 | 15 | 8 | 871 | 53 | 84 | 2.08 | 36 | 2.6 | 0.71 |
| 20 | 3.0 | 0.71 | 02 | 0 | 500 | 1020 | 15 | 8 | 870 | 53 | 81 | 2.17 | 32 | 3.0 | 0.74 |
| 21 | 3.0 | 0.71 | 02 | 0 | 450 | 1050 | 23 | 7 | 912 | 53 | 85 | 2.16 | 39 | 2.9 | 084 |
| 22 | 3.0 | 0.71 | 02 | 0 | 500 | 1050 | 17 | 8 | 905 | 53 | 82 | 2.29 | 30 | 2.4 | 0.66 |
| 23 | 3.0 | 0.71 | 0.2 | 0.1 Mg | 450 | 1020 | 18 | 6 | 934 | 50 | 89 | 2.04 | 34 | 4.6 | 0.70 |
| 24 | 3.0 | 0.71 | 02 | 0.1 Mg | 500 | 1020 | 15 | 7 | 927 | 50 | 88 | 2.08 | 30 | 3.4 | 0.83 |
| 25 | 3.0 | 0.71 | 02 | 0.1 Mg | 450 | 1050 | 21 | 7 | 948 | 49 | 90 | 2.11 | 30 | 2.5 | 0.66 |
| 26 | 3.0 | 071 | 02 | 01 Mg | 500 | 1050 | 15 | 5 | 948 | 49 | 89 | 2.33 | 39 | 2.2 | 067 |
| 27 | 3.0 | 0.71 | 0 | 0.5Sn | 500 | 1020 | 17 | 8 | 885 | 46 | 84 | 2.08 | 29 | 1.7 | 0.72 |
| 28 | 3.0 | 0.71 | 0 | 0.5Zn | 500 | 1020 | 19 | 6 | 886 | 48 | 81 | 2.18 | 29 | 3.4 | 0.72 |
| 29 | 3.0 | 0.71 | 0 | 01 Ag | 500 | 1020 | 16 | 6 | 874 | 49 | 87 | 2.26 | 33 | 29 | 0.34 |
| 30 | 3.0 | 0.71 | 02 | 0.5Sn | 500 | 1020 | 17 | 8 | 888 | 51 | 87 | 2.04 | 33 | 2.4 | 071 |
| 31 | 3.0 | 0.71 | 0.2 | 0.5Zn | 500 | 1020 | 16 | 6 | 880 | 49 | 84 | 2.12 | 37 | 3.8 | 0.74 |
| 32 | 3.0 | 0.71 | 02 | 0.1 Ag | 500 | 1020 | 17 | 5 | 878 | 52 | 83 | 2.09 | 31 | 3.3 | 0.78 |
| 33 | 3.8 | 0.90 | 0 | 0 | 450 | 1050 | 16 | 9 | 952 | 45 | 85 | 2.34 | 35 | 3.6 | 066 |
| 34 | 3.8 | 0.80 | 0 | 0 | 500 | 1050 | 16 | 9 | 946 | 44 | 83 | 2.44 | 37 | 3.2 | 0.58 |
| 35 | 3.8 | 0.90 | 0.2 | 0 | 450 | 1050 | 16 | 7 | 967 | 48 | 82 | 2.39 | 38 | 3.4 | 0.64 |
| 36 | 3.8 | 090 | 02 | 0 | 500 | 1050 | 16 | 6 | 961 | 47 | 82 | 2.44 | 29 | 3.1 | 0.60 |

**(Table 2-1)**

| No. | composition(mass%) | | | | aging temperature (°C) | solution treatment temperature (°C) | average grain size (*µ*m) | max grain size -min grain size (*µ*m) | average strength (MPa) | average electrical conductivity (%IACS) | average stress relaxation performance (%) | average roughness of bending (*µ*m) | variability of strength (MPa) | variability of stress relaxation performance (%) | variability of roughness of bending (*µ*m) |
|---|---|---|---|---|---|---|---|---|---|---|---|---|---|---|---|
| | Co | Si | Or | others | | | | | | | | | | | |
| 37 | 0.7 | 0.17 | 0 | 0 | - | 950 | 24 | 16 | 659 | 58 | 81 | 3.58 | 48 | 5.0 | 1.40 |
| 38 | 2.0 | 0.48 | 0 | 0 | - | 1020 | 32 | 20 | 765 | 57 | 83 | 3.24 | 57 | 6.4 | 1.46 |
| 39 | 3.0 | 0.71 | 0 | 0 | - | 1020 | 22 | 12 | 849 | 53 | 86 | 3.03 | 55 | 5.6 | 1.96 |
| 40 | 3.0 | 0.71 | 0 | 0 | - | 1050 | 36 | 36 | 830 | 51 | 85 | 3.12 | 51 | 5.8 | 1.99 |
| 41 | 3.0 | 0.71 | 0 | 0 | - | 1070 | 50 | 44 | 807 | 52 | 87 | 3.34 | 50 | 4.6 | 2.01 |
| 42 | 3.0 | 0.71 | 0.2 | 0 | - | 1020 | 22 | 14 | 847 | 54 | 84 | 310 | 48 | 5.5 | 1.87 |
| 43 | 3.0 | 0.71 | 0.2 | 0 | - | 1050 | 32 | 21 | 830 | 53 | 83 | 2.94 | 43 | 4.2 | 1.92 |
| 44 | 30 | 0.71 | 0.2 | 0 | - | 1070 | 46 | 33 | 817 | 53 | 86 | 3.38 | 52 | 6.1 | 2.14 |
| 45 | 3.0 | 0.71 | 0 | 0 | - | 950 | 9 | 8 | 777 | 55 | 76 | 2.05 | 39 | 4.1 | 1.13 |
| 46 | 3.0 | 0.71 | 0 | 0 | - | 900 | 7 | 4 | 743 | 59 | 77 | 2.05 | 35 | 3.3 | 1.09 |
| 47 | 3.0 | 0.71 | 02 | 0 | - | 950 | 8 | 7 | 792 | 54 | 76 | 1.96 | 38 | 4.5 | 1.30 |
| 48 | 3.0 | 0.71 | 0.2 | 0 | - | 900 | 6 | 4 | 753 | 57 | 73 | 1.90 | 38 | 3.6 | 1.15 |
| 49 | 3.0 | 0.71 | 0 | 0 | 300 | 1020 | 21 | 19 | 834 | 52 | 83 | 2.95 | 62 | 5.4 | 1.40 |
| 50 | 3.0 | 0.71 | 0 | 0 | 300 | 1050 | 34 | 28 | 837 | 52 | 85 | 3.06 | 52 | 4.8 | 1.46 |

**(Table 2-2)**

| No. | composition(mass%) | | | | aging temperature (°C) | solution treatment temperature (°C) | average grain size (*µ*m) | max grain size -mln grain size (*µ*m) | average strength (MPa) | average electrical conductivity (%IACS) | average stress relaxation performance (%) | average roughness of bending (*µ*m) | variability of strength (MPa) | variability of stress relaxation performance (%) | variability of roughness of bending (*µ*m) |
|---|---|---|---|---|---|---|---|---|---|---|---|---|---|---|---|
| | Co | Si | Cr | others | | | | | | | | | | | |
| 51 | 3.0 | 0.71 | 0 | 0.1 Mg | 300 | 1020 | 20 | 21 | 882 | 51 | 83 | 3.14 | 63 | 5.1 | 2.04 |
| 52 | 3.0 | 0.71 | 0 | 0.1 Mg | 300 | 1050 | 31 | 35 | 868 | 49 | 82 | 2.97 | 59 | 4.9 | 1.50 |
| 53 | 3.0 | 0.71 | 0.2 | 0 | 300 | 1020 | 19 | 15 | 839 | 51 | 83 | 2.95 | 57 | 5.3 | 1.11 |
| 54 | 3.0 | 0.71 | 0.2 | 0 | 300 | 1050 | 29 | 22 | 845 | 51 | 82 | 2.92 | 55 | 4.4 | 1.83 |
| 55 | 4.7 | 1.12 | 0 | 0 | 450 | 1020 | 14 | 11 | 780 | 38 | 81 | 2.31 | 46 | 5.5 | 1.41 |
| 56 | 4.7 | 1.12 | 0.2 | 0 | 450 | 1020 | 15 | 9 | 795 | 40 | 85 | 2.31 | 52 | 5.8 | 1.38 |
| 57 | 3.0 | 0.71 | 0 | 0 | 550 | 1020 | 28 | 19 | 860 | 50 | 81 | 2.10 | 54 | 5.0 | 082 |
| 58 | 3.0 | 0.71 | 0 | 0 | 550 | 1050 | 34 | 25 | 888 | 51 | 82 | 2.36 | 60 | 4.9 | 1.29 |
| 59 | 3.0 | 0.71 | 0 | 0.1 Mg | 550 | 1020 | 23 | 18 | 900 | 48 | 80 | 2.24 | 71 | 6.4 | 1.18 |
| 60 | 3.0 | 0.71 | 0 | 0.1 Mg | 550 | 1050 | 31 | 22 | 926 | 50 | 82 | 2.66 | 72 | 5.4 | 1.42 |
| 61 | 3.0 | 0.71 | 02 | 0 | 550 | 1020 | 25 | 25 | 866 | 52 | 83 | 2.06 | 60 | 6.2 | 1.10 |
| 62 | 3.0 | 0.71 | 02 | 0 | 550 | 1050 | 29 | 27 | 897 | 51 | 85 | 2.40 | 69 | 6.4 | 1.06 |
| 63 | 3.0 | 0.71 | 0.2 | 0.1 Mg | 550 | 1020 | 27 | 20 | 906 | 50 | 84 | 2.17 | 72 | 5.4 | 1.02 |
| 64 | 3.0 | 0.71 | 0.2 | 0.1 Mg | 550 | 1050 | 31 | 21 | 935 | 50 | 83 | 2.67 | 62 | 5.9 | 1.62 |

Alloys of No.1, 5 and 6 are working examples according to the present invention wherein concentrations of Co are relatively low (0.7 and 0.2 mass%). Those average strengths are low because of low concentrations of Co and variabilities of all kinds of characteristics are small. Alloys 2, 3 and 4 are comparative examples.

Alloys of No.9 to 11, 13 to 15, 18, 21, 23 to 26, 28, 29, 31, 32, 35 and 36 are working examples according to the present invention wherein concentrations of Co are high (not less than 3.0 mass%). All of them have appropriate strength and electrical conductivity for electronic materials and variabilities of all kinds of characteristics are small. Alloys 7, 8, 12,16, 17,19, 20, 22, 27, 30, 33 and 34 are comparative examples.

With respect to alloys of No.37 to 44, strength and bending workability deteriorated because the first aging treatment was not conducted and then the grain size increased in the solution treatment.

With respect to alloys of No.45 to 48, strength and stress relaxation characteristics deteriorated because the first aging treatment was not conducted and the temperature of the solution treatment was low, and then the second-phase particles did not form into a solid solution sufficiently and the grain size was too small.

With respect to alloys of No.49 to 54, strength and bending workability deteriorated because the temperature of the solution treatment was too low and number of the second-phase particles was small, and then grain size increased in the solution treatment. Further, variability of grain size increased, and then variability of characteristics increased.

With respect to alloys of No.55 to 56, strength and electrical conductivity deteriorated because additive amount of Co was too large.

With respect to alloys of No.57 to 64, variability of grain size increased because the temperature of the first aging treatment was too high and then the second-phase particles grew ununiformly. As a result, variability of characteristics increased.

## Claims

1. A copper alloy for electronic materials, containing 0.5 to 4.0 mass% Co, 0.1 to 1.2 mass% Si, the balance being Cu and unavoidable impurities,
- optionally containing Cr in a maximum amount of 0.5 mass%,
- optionally containing a single element or two or more elements selected from Mg, Mn, Ag and P in total in a maximum amount of 0.5 mass%,
- optionally containing one or two elements selected from Sn and Zn in total in a maximum amount of 2.0 mass%,
- optionally containing a single element or two or more elements selected from As, Sb, Be, B,Ti, Zr, Al and Fe in total in a maximum amount of 2.0 mass%,
wherein an average grain size is 15 to 30 µm and an average difference between maximum grain size and minimum grain size in every observation field of 0.5 mm² is not more than 7 µm, wherein the average difference between maximum grain size and minimum grain size is the mean value of the differences in 15 observation fields.

2. A method for manufacturing the copper alloy according to claim 1, comprising sequentially conducting:
- step 1 for casting an ingot having a desired composition;
- step 2 for heating the ingot for not less than 1 hour at 950 °C to 1050 °C, thereafter hot rolling the ingot, setting the temperature to not less than 850 °C when hot rolling is completed, and cooling the ingot at an average cooling rate being not less than 15 °C/s from 850 °C to 400 °C;
- step 3 for cold rolling at a reduction ratio being not less than 70 %;
- step 4 for conducting aging by heating at 350 °C to 500 °C for 1 to 24 hours;
- step 5 for conducting a solution treatment at 950 °C to 1050 °C, for 60 to 300 seconds at not less than 950 °C to less than 1000 °C, and for 30 to 180 seconds at not less than 1000 °C to less than 1050 °C, and cooling the material at an average cooling rate being not less than 15 °C/s when the material temperature is reduced from 850 °C to 400 °C;
- step 6 for conducting optional cold rolling;
- step 7 for conducting aging; and
- step 8 for conducting optional cold rolling.

3. A copper alloy product using the copper alloy of claim 1.

4. An electronic component using the copper alloy of claim 1.

## Patentansprüche

1. Eine Kupferlegierung für elektronische Materialien, enthaltend 0.5 bis 4.0 Massenprozent Co, 0.1 bis 1.2 Massenprozent Si, wobei der Restgehalt Cu und unvermeidbare Verunreinigungen sind,
- gegebenenfalls enthaltend Cr in einer Höchstmenge von 0.5 Massenprozent,
- gegebenenfalls enthaltend ein einzelnes oder zwei oder mehrere Elemente ausgewählt aus Mg, Mn, Ag und P insgesamt in einer Höchstmenge von 0.5 Massenprozent,
- gegebenenfalls enthaltend ein oder zwei Elemente ausgewählt aus Sn und Zn in einer Höchstmenge von insgesamt 2.0 Massenprozent,
- gegebenenfalls enthaltend ein einzelnes oder zwei oder mehrere Elemente ausgewählt aus As, Sb, Be, B,Ti, Zr, Al und Fe in einer Höchstmenge von insgesamt 2.0 Massenprozent,
wobei eine durchschnittliche Korngröße von 15 bis 30 µm beträgt und eine durchschnittliche Differenz zwischen maximaler Korngröße und minimaler Korngröße in jedem Betrachtungsfeld von 0.5 mm² nicht mehr als 7 µm beträgt, wobei die durchschnittliche Differenz zwischen maximaler Korngröße und minimaler Korngröße der Mittelwert der Differenzen in 15 Betrachtungsfeldern ist.

2. Ein Verfahren zur Herstellung der Kupferlegierung gemäß Anspruch 1, umfassend die sequenzielle Durchführung von:
- Schritt 1 zum Gießen eines Barrens welcher eine gewünschte Zusammensetzung aufweist;
- Schritt 2 zum Erhitzen des Barrens für nicht weniger als 1 Stunde bei nicht weniger als 950 °C bis 1050 °C, anschließendem Warmwalzen des Barrens, wobei die Temperatur bei Abschluss des Warmwalzen des Barrens auf nicht weniger als 850 °C eingestellt wird, und Abkühlen des Barrens mit einer durchschnittlichen Kühlungsrate von nicht weniger als 15 °C/s von 850 °C auf 400 °C;
- Schritt 3 zum Kaltwalzen mit einem Reduktionsverhältnis von nicht weniger als 70 %;
- Schritt 4 zur Durchführung einer Alterung durch Erhitzen bei 350 °C bis 500 °C für 1 bis 24 Stunden;
- Schritt 5 zur Durchführung einer Lösungsglühung bei 950 °C bis 1050 °C, für 60 bis 300 Sekunden bei nicht weniger als 950 °C bis weniger als 1000 °C, und für 30 bis 180 Sekunden bei nicht weniger als 1000 °C bis weniger als 1050 °C, und Abkühlen des Materials mit einer durchschnittlichen Kühlungsrate von nicht weniger als 15 °C/s während die Materialtemperatur von 850 °C auf 400 °C reduziert wird;
- Schritt 6 zur optionalen Durchführung einer Kaltwalzung;
- Schritt 7 zur Durchführung einer Alterung; und
- Schritt 8 zur optionalen Durchführung einer Kaltwalzung.

3. Ein Kupferlegierungsprodukt welches die Kupferlegierung gemäß Anspruch 1 nutzt.

4. Eine elektronische Komponente welche die Kupferlegierung gemäß Anspruch 1 nutzt.

## Revendications

1. Alliage de cuivre pour matériaux électroniques, contenants de 0,5 à 4,0 % en masse de Co, 0,1 à 1,2 % en masse de Si, le complément étant Cu et des impuretés inévitables,
- contenant facultativement Cr en une quantité maximale de 0,5 % en masse ;
- contenant facultativement un élément unique ou deux éléments ou plus choisis parmi Mg, Mn, Ag et P au total en une quantité maximale de 0,5 % en masse ;
- contenant facultativement un ou deux éléments choisis parmi Sn et Zn au total en une quantité maximale de 2,0 % en masse,
- contenant facultativement un élément unique ou deux éléments ou plus choisis parmi As, Sb, Be, B, Ti, Zr, Al et Fe au total en une quantité maximale de 2,0 % en masse,
dans lequel une taille de grain moyenne est de 15 à 30 µm et une différence moyenne entre la taille de grain maximale et la taille de grain minimale dans chaque champ d'observation de 0,5 mm² n'est pas supérieure à 7 µm, dans lequel la différence moyenne entre la taille de grain maximale et la taille de grain minimale est la valeur moyenne des différences dans 15 champs d'observation.

2. Procédé de fabrication de l'alliage de cuivre selon la revendication 1, comprenant la conduite séquentielle de :
- l'étape 1 pour couler un lingot ayant une composition souhaitée ;
- l'étape 2 pour chauffer le lingot pendant pas plus de 1 heure à 950 °C à 1050 °C, puis laminer à chaud le lingot, régler la température à pas moins de 850 °C une fois que le laminage à chaud est achevé, et refroidir le lingot à une vitesse de refroidissement moyenne n'étant pas inférieure à 15 °C/s de 850 °C à 400 °C ;
- l'étape 3 pour laminer à froid à un rapport de réduction n'étant pas inférieur à 70 % ;
- l'étape 4 pour conduire un vieillissement par chauffage à 350 °C à 500 °C pendant 1 à 24 heures ;
- l'étape 5 pour conduire un traitement en solution à 950 °C à 1050 °C pendant 60 à 300 secondes à pas moins de 950 °C à moins de 1000 °C, et pendant 30 à 180 secondes à pas moins de 1000 °C à moins de 1050 °C, et refroidir le matériau à une vitesse de refroidissement moyenne n'étant pas inférieure à 15 °C/s lorsque la température du matériau est réduite de 850 °C à 400 °C ;
- l'étape 6 pour conduire un laminage à froid facultatif ;
- l'étape 7 pour conduire un vieillissement ; et
- l'étape 8 pour conduire un laminage à froid facultatif.

3. Produit d'alliage de cuivre utilisant l'alliage de cuivre de la revendication 1.

4. Composant électronique utilisant l'alliage de cuivre de la revendication 1.
